

# UNITED STATES PATENT OFFICE.

JOHN T. H. DEMPSTER, OF SCHENECTADY, NEW YORK, ASSIGNOR TO GENERAL ELECTRIC COMPANY, A CORPORATION OF NEW YORK.

## PROTECTIVE COVERING FOR RESISTANCE-CONDUCTORS.

1,028,444.

Specification of Letters Patent.

Patented June 4, 1912.

No Drawing.

Application filed March 20, 1909. Serial No. 484,772.

*To all whom it may concern:*

Be it known that I, JOHN T. H. DEMPSTER, a citizen of the United States, residing at Schenectady, county of Schenectady, 5 State of New York, have invented certain new and useful Improvements in Protective Coverings for Resistance-Conductors, of which the following is a specification.

This invention relates to means for protecting resistance conductors which are used in electric heaters and the like and has for its object the provision of a covering or protective layer which will prevent the injurious action of certain resistance conductors, 15 when heated, upon the insulating material which is in contact therewith.

In the construction of electric heaters and the like, high resistance conductors are frequently used containing metal which forms 20 an oxid on the conductor. This oxid has been found in some cases to attack the mica or other insulating material which is placed in contact with it when the conductor attains a high temperature. This is particularly true of certain resistance conductors 25 containing iron, as for instance, an alloy of iron, nickel, and chromium. A resistance conductor of this composition, when heated, forms an oxid or scale which has been found to combine with mica to form a 30 very low melting point mixture. I have found that by applying a coating of a mixture which is basic in character this action between the oxid and the mica can be prevented.

In carrying out my invention, I apply preferably to the surface of the mica, although of course the coating may be applied to the resistance conductor, a coating composed of a basic oxid with an aluminate and a binder. This binder may be of such a nature as to make a glutinous mixture like paint, so that the material may be laid on with a brush. The particular composition 45 which I have found to be very satisfactory is a mixture of 50% of an oxid of aluminum, magnesium, zinc, or chromium and 50% sodium aluminate. This is mixed with enough dextrin and water to

make a thick cement or paste. The components of this compound, being basic in character, will not slag with the oxid on the conductor. The sodium aluminate reduces the melting point somewhat, which is still very high, and the dextrin furnishes a small 55 amount of carbon when heated and prevents the initial oxidation of the conductor.

It is evident of course, that other materials may be used and the proportions varied, if desired, since I have merely set 60 forth a particular and specific compound in accordance with the patent statutes for purposes of illustration, and various modifications thereof will suggest themselves to those skilled in the art without departing 65 from the spirit of my invention, the scope of which is set forth in the annexed claims.

What I claim as new and desire to secure by Letters Patent of the United States, is,—

1. The combination of an oxidizable resistance conductor, a mica insulation adjacent thereto, and a protective material interposed between the conductor and the mica, said material comprising a basic oxid.

2. The combination of an oxidizable resistance conductor, a mica insulation adjacent thereto, and a protective material interposed between the conductor and the mica, said material comprising aluminum oxid and an aluminate.

3. The combination of an oxidizable resistance conductor, a mica insulation adjacent thereto, and a protective material interposed between the conductor and the mica, said material comprising aluminum oxid, an aluminate and a binder.

4. The combination of a resistance conductor containing iron, nickel, and chromium, a mica insulation adjacent thereto, and a protective material between the conductor and the mica, said material comprising aluminum oxid and an aluminate.

In witness whereof, I have hereunto set my hand this 19th day of March, 1909.

JOHN T. H. DEMPSTER.

Witnesses:

HELEN ORFORD,  
MARGARET E. WOOLLEY.